# EUROPEAN PATENT SPECIFICATION

(11) **EP 0 826 512 B1**
(45) Date of publication and mention of the grant of the patent: **22.03.2000**
(21) Application number: 97114863.0
(22) Date of filing: 27.08.1997
(51) Int. Cl.: B41M 5/38, B41M 5/40

(54) **Thermal transfer recording material heving an intermediate adhesive layer**
Thermisches Übertragungsaufzeichnungsmaterial mit einer Klebstoffzwischenschicht
Matériau pour l'enregistrement par transfert thermique ayant une couche intermédiaire adhésive

(30) Priority: 28.08.1996 JP 22678596
(43) Date of publication of application: 04.03.1998
(73) Proprietor: FUJICOPIAN CO., LTD., Osaka-shi, Osaka-fu (JP)
(72) Inventor: Shinohara Tomohiro, c/o Fujicopian Co., Ltd., Nishiyodogawa-ku, Osaka-shi, Osaka-fu (JP); Arimura, Takao, c/o Fujicopian Co., Ltd., Nishiyodogawa-ku, Osaka-shi, Osaka-fu (JP); Kurokawa, Kenji, c/o Fujicopian Co., Ltd., Nishiyodogawa-ku, Osaka-shi, Osaka-fu (JP)
(74) Representative: Tiedtke, Harro, Dipl.-Ing.

(56) References cited:
- EP-A- 0 363 929
- EP-A- 0 410 724
- PATENT ABSTRACTS OF JAPAN vol. 14, no. 379 (M-1012), 16 August 1990 & JP 02 141286 A (FUJITSU LIMITED), 30 May 1990,
- PATENT ABSTRACTS OF JAPAN vol. 10, no. 378 (M-546), 17 December 1986 & JP 61 169283 A (FUJITSU LIMITED), 30 July 1986,
- PATENT ABSTRACTS OF JAPAN vol. 10, no. 66 (M-461), 15 March 1986 & JP 60 212393 A (FUJITSU K.K.), 24 October 1985,

## Description

The present invention relates to a thermal transfer recording medium. More particularly, it relates to a thermal transfer recording medium which does not cause the so-called "ink-falling" and is capable of providing printed images with high definition.

Recently thermal transfer recording system has been widely applied because thermal transfer printers used therein have characteristics such as easy maintenance, availability of small-sized and lightweight ones and low-cost.

In such a thermal transfer recording system, respective plural heating elements (dots) of a thermal head are allowed to selectively generate heat in response to picture signals, thereby selectively transferring the heat-meltable ink layer of a thermal transfer recording medium in dots to give a printed image on a receptor. Therefore, improved dot-reproducibility is required to obtain printed images with high definition. This dot-reproducibility refers to the coincidence of the shape of dots of the transferred heat-meltable ink with that of the heating elements.

Measures for improving the dot-reproducibility include selection of a heat-meltable material showing a sharp peak in its DSC (differential scanning calorimetry) curve for the vehicle of the heat-meltable ink layer. For example, carnauba wax (penetration: 1), which is a very hard wax, was used as a vehicle of the heat-meltable ink layer, as a result of further consideration given to the scratch resistance of printed images and the like. A heat-meltable ink layer containing carnauba wax as a vehicle thereof offers printed images with improved dot-reproduction because the wax shows a sharp peak in its DSC curve. However, the incorporation of a large amount of carnauba wax into a heat-meltable ink layer results in a problem that the so-called "ink-falling" phenomenon occurs. The term "ink-falling" refers to a phenomenon in which, during traveling of the thermal transfer recording medium, which is loaded in a cassette, in a thermal transfer printer, portions of the heat-meltable ink layer are peeled off from the foundation when the recording medium comes into sliding contact with guide members of the cassette, the thermal head, etc. and, hence, is subjected to external force. The ink-falling phenomenon is remarkable in using the recording medium in low-temperature environments.

The ink-falling phenomenon is undesirable because portions of the recording medium wherein the ink layer is peeled off cannot be used to form printed images and the generated ink powder is accumulated in the thermal head, resulting in a decrease in image quality or contamination in the inside of the printer.

Conventional measures for preventing the ink-falling phenomenon include (1) a method wherein the content of a resin component in the heat-meltable ink layer is increased to improve adhesion of the ink layer, and (2) another method wherein a wax having a greater penetration is used in combination with carnauba wax to impart flexibility or softness to the heat-meltable ink layer. However, the method (1) involves a problem that the viscosity of an ink coating liquid is increased with increasing content of the resin component and, hence, the application property of the coating liquid becomes poor, resulting in failure to form a uniform ink layer. The method (2) involves a problem that during exchange of the recording medium in using it in low-temperature environment, the ink thereof sticks to the hand.

EP-A-0 363 929 discloses a thermal imprint ink sheet having a film substrate, an adhesive layer formed on the film substrate and an ink layer formed on the adhesive layer wherein the adhesive layer comprises a mixture of a first polyester resin and a second polyester resin, the first polyester resin having a first glass transition temperature (Tg) higher than environmental temperatures at which the ink sheet is used and the second polyester resin having a second glass transition temperature (Tg) lower than said environmental temperature. It is mentioned that a single polyester resin in the adhesive layer is not practically usable.

EP-A-0 410 724 discloses a heat-transfer image recording medium comprising a support, a heat-transfer layer provided on the support and a non-transfer layer which is interposed between the support and the transfer layer. The non-transfer layer comprises a mixture of two thermoplastic polymers selected from specific structural classes.

In view of the foregoing, an object of the present invention is to provide a thermal transfer recording medium which causes no ink-falling in low-temperature environments and exerts excellent dot-reproducibility to form printed images with high definition.

This and other objects of the present invention will become apparent from the description hereinafter.

The present invention provides a thermal transfer recording medium comprising a substrate (also called foundation) having thereon a heat-meltable ink layer, and an intermediate adhesive layer provided between the substrate and the heat-meltable ink layer, the intermediate adhesive layer comprising 20 to 80 % by weight of a resin component consisting of one polyester resin having a glass transition temperature of not higher than 20°C, and 20 to 80 % by weight of at least one component selected from a pigment and carbon black.

In an embodiment of the present invention, the polyester resin has a glass transition temperature of not higher than 0°C.

In another embodiment of the present invention, the heat-meltable ink layer comprises a coloring agent and a vehicle, the vehicle comprising not less than 40 % by weight of caranuba wax.

In still another embodiment of the present invention, the vehicle comprises not less than 50 % by weight of carnauba wax.

In a further embodiment of the present invention, the intermediate adhesive layer comprises 40 to 70 % by weight of a polyester resin having a glass transition temperature of not higher than 20°C and 30 to 60 % by weight of at least one component selected from of a pigment and carbon black.

Fig. 1 is a schematic view illustrating a measuring device for examining the ink-falling of a thermal transfer recording medium.

The thermal transfer recording medium of the present invention is characterized in that between the foundation and the heat-meltable ink layer is provided an intermediate adhesive layer comprising 20 to 80 % by weight of a resin component consisting of one polyester resin having a glass transition temperature of not higher than 20°C, and 20 to 80 % by weight of at least one component selected from a pigment and carbon black.

In the present invention, the intermediate adhesive layer maintains flexibility or softness even in low-temperature environments wherein the temperature is lower than normal temperature because one polyester resin having a glass transition temperature of not higher than 20°C is used as the resin component and, hence, serves as some type of a buffer layer between the foundation and the heat-meltable ink layer, thereby causing no ink-falling even in the case that the heat-meltable ink layer is relatively hard. The use of the polyester resin having a glass transition temperature of higher than 20°C as the resin component for the intermediate adhesive layer results in ink-falling because the polyester resin crystallizes in low-temperature environments and the function of the intermediate adhesive layer as a buffer layer is lost. From the viewpoint of retaining the flexibility or softeness of the intermediate adhesive layer in low-temperature environments, a polyester resin having a glass transition temperature of not higher than 0°C is preferable.

In the present invention, the intermediate adhesive layer is incorporated with at least one of a pigment and carbon black (hereinafter, in some cases, referred to as "particulate material") in addition to the polyester resin. The incorporation of the particulate material produces fine unevenness on the surface of the intermediate adhesive layer to increase the contact area between the intermediate adhesive layer and the heat-meltable ink layer. As a result, the ink-falling can be more sufficiently prevented.

The intermediate adhesive layer in accordance with the present invention contains 20 to 80 % by weight, preferably 40 to 70 % by weight, of a resin component consisting of one polyester resin having a glass transition temperature of not higher than 20°C, and 20 to 80 % by weight, preferably 30 to 60 % by weight, of a particulate material. When the content of the polyester resin having a glass transition temperature of not higher than 20°C is lower than the above range or the content of the particulate material is higher than the above range, the function of the intermediate adhesive layer as a buffer layer is degraded to fail to sufficiently exert the effect of preventing the ink-falling and a problem that the application property of a coating liquid for the intermediate adhesive layer is degraded is further invited. When the content of the polyester resin is higher than the above range or the content of the particulate material is lower than the above range, the contact area between the intermediate adhesive layer and the ink layer is not increased due to the lower content of the particulate material to fail to sufficiently exert the effect of preventing the ink-falling and the so-called "layer-like transfer" which refers to the phenomenon wherein an excess portion of the ink layer that is not heated during the thermal transfer is also transferred, is prone to further occur, resulting in deterioration of the dot-reproducibility.

As the aforesaid polyester resin there can be used linear saturated polyester resins which are obtained by polycondensation of a dibasic acid and a diol compound and have a glass transition temperature of not higher than 20°C, preferably not higher than 0°C. Examples of the dibasic acid are adipic acid, azelaic acid, sebacic acid, phthalic acid and Het acid (chlorendic acid). These dibasic acids can be used either alone or in combinations of two or more species thereof. Examples of the diol compounds are ethylene glycol, propylene glycol, 1, 4-butanediol, 1, 6-hexanediol, 1, 4-cyclohexanedimethanol, hydrogenated bisphenol A and dibromoneopentylene glycol. These diol compounds can be used either alone or in combinations of two or more species thereof.

Examples of pigments as the particulate material are silica, calcium carbonate, magnesium carbonate, barium sulfate and aluminium silicate. These pigments can be used either alone or in combinations of two or more species thereof.

The pigment and carbon black may be used either alone or in combiantion as the particulate material. From the viewpoint of producing fine unevenness on the surface of the intermediate adhesive layer, the particulate material preferably has an average particle size of 0.5 to 10 µm.

The intermediate adhesive layer may be incorporated with a small amount of a dispersing agent or the like in addition to the aforesaid ingredients.

The thickness of the intermediate adhesive layer is preferably from 0.3 to 1.0 µm from the viewpoint of the adhesiveness and the transfer sensitivity.

The intermediate adhesive layer can be formed by applying onto a foundation a coating liquid which is prepared by dissolving or dispersing the polyester resin and the particulate material into an appropriate solvent, followed by drying.

As the heat-meltable ink layer in accordance with the present invention there can be used conventional ones without particular limitation so long as they are one-time type heat-meltable ink layers each comprising a coloring agent and a heat-meltable vehicle as main ingredients. However, preferred is a heat-meltable ink layer whose vehicle component contains not less than 40 % by weight, especially not less than 50 % by weight, of carnauba wax to form printed images having excellent durability with excellent dot-reproducibility as well as to prevent the ink-falling in combination with the aforesaid intermediate adhesive layer. When the content of carnauba wax in the vehicle component is lower than the above range, the dot-reproducibility is prone to be deteriorated to fail to produce printed images with high definition and the durability of printed images is also prone to be decreased.

Usable as the vehicle component other than carnauba wax are waxes other than carnauba wax and/or resins. As the waxes there can be appropriately selected and used those conventionally used in this field, such as paraffin wax, microcrystalline wax, oxidized wax, ester wax, candelilla wax, rice wax and montan wax. As the resins there can be appropriately selected and used those conventionally used in this field, such as polyethylene, ethylene-vinyl acetate resin, polyamide resins, polyester resins, epoxy resins and acrylic resins.

Carbon black as well as usual pigments and dyes can be appropriately selected and used as the coloring agent.

Suitable ranges for the contents of the foregoing ingredients in the heat-meltable ink layer in accordance with the present invention are as follows:

| Ingredient | % by weight |
|---|---|
| Carnauba wax | 40 to 95 (preferably 50 to 90) |
| Other waxs | 0 to 40 (preferably 10 to 30) |
| Resin | 0 to 40 (preferably 10 to 30) |
| Coloring agent | 5 to 20 |

The heat-meltable ink layer in accordance with the present invention can be formed by applying an ink of the foregoing formulation onto the aforesaid intermediate adhesive layer by means of a hot-melt coating method or a solvent coating method. The thickness of the heat-meltable ink layer is preferably from 1 to 5 µm from the viewpoint of the optical density of images and the transfer sensitivity.

In the present invention, as required, an overcoat layer may be provided on the heat-meltable ink layer. The overcoat layer is provided for the purpose of preventing smearing or the like. Usually the overcoat layer is an uncolored layer comprising a wax as a main ingredient.

Usable as the foundation in the present invention are highly heat-resistant plastic films such as polyethylene terephthalate film, polycarbonate films, polyimide films and nylon films, and cellophane, parchment paper and condenser paper. The thickness of the foundation is usually from 2 to 10 µm, preferably from 3.5 to 6 µm. From the viewpoint of good adhesion to the intermediate adhesive layer, polyethylene terephthalate film is especially preferred.

As required, on the back side (the side adapted to come into slide contact with a thermal head) of the foundation may be formed a heat-resistant layer comprising one or more resins selected from silicone resins, fluorine-containing resins, acrylic resins, epoxy resins, phenol resins, cellulose resins, and the like.

The present invention will be more fully described by way of Examples and Comparative Examples. It is to be understood that the present invention is not limited to the Examples, and various changes and modifications may be made in the invention without departing from the scope thereof.

### Examples 1 to 3 and Comparative Examples 1 to 3

Into a mixed solvent of toluene methyl ethyl ketone was added each composition for intermediate adhesive layer of the formulation shown in Table 1 so that the total solid concentration became 10 % by weight. The resulting mixture was agitated at a high speed in an attritor for 60 minutes to give a coating liquid for intermediate adhesive layer. Onto one side of a 6 µm-thick polyethylene terephthalate film which was provided on the other side thereof with a heat-resistant layer composed of a silicone resin was applied the coating liquid by means of a solvent coater so that the coating amount after drying was 0.5·10⁻³ kg/m², followed by drying to give an intermediate adhesive layer. In Comparative Example 3, the resulting coating liquid failed to form a uniform layer due to its poor application property and, hence, subsequent treatments were not performed.

Each composition for heat-meltable ink layer of the formulation shown in Table 1 was sufficiently kneaded by means of a 3-roll mill to give a heat-meltable ink. The ink was applied in a coating amount of 3.0·10⁻³kg/m² onto the intermediate adhesive layer by means of a hot-melt coater to give a heat-meltable ink layer.

Each of the thus obtained thermal transfer recording media was evaluated for dot-reproducibility and ink-falling. The results are shown in Table 1.

### 〈Dot-reproducibility〉

Each of the thermal transfer recording media was used to form a printed image under the printing conditions mentioned below. The printed image was observed with a metallograph (XF(U)NR, trade name made by NIKON CORPORATION) at a magnification of 50 to determine the ratio of the area of one dot of the image to that of one dot of the heating elements (area of one dot of the image/area of one dot of the heating elements). The dot-reproducibility was evaluated according to the following criterion:

| Printing conditions: | |
|---|---|
| Thermal printer | line printer (B-30 made by TEC Corporation |
| Thermal head | line head type |
| Head pressure | 0.7 kg/25.4 mm (1 inch) |
| Printing energy | 19.0 mJ/mm² |
| Printing speed | 0.102 m (4 inches)/second |
| Receptor paper | TPKB trade name (Bekk smoothness: 200 seconds) |

### Evaluation criterion:

3 . . . Area ratio: 0.95 to 1.05
2... Area ratio: 0.90 to less than 0.95
1... Area ratio: less than 0.90

### 〈Ink-falling〉

With respect to each of the thermal transfer recording media, the degree of ink-falling was examined in a low-temperature environment (dry room at 0°C ) with use of a measuring device as shown in Fig. 1. This test is a substitute for a test for examining the degree of ink-falling when the thermal transfer recording medium is squeezed through a thermal head.

As shown in Fig. 1, a glass plate 3 was fixed to a support member 2 which was mounted on a table 1 with projecting out from an edge of the table 1. A ribbon-like thermal transfer recording medium 4 (width: 12.7 mm) was arranged so that it lay upward on the ink layer side and was brought into contact with the end surface of the glass plate 3 on the back side thereof. A weight 5 was attached to one end of the recording medium that hung down and a movable member 6 was attached to the other end of the recording medium. In such a state, the movable member 6 was moved at a speed of 0.0217 m/s in the direction indicated by the arrow to examine whether the ink-falling occurred. This examination operation was repeated while successively replacing the weight 5 with a heavier one by 0.05 kg within the range of 0.05 to 0.3 kg. The ink-falling was evaluated according to the following criterion:

### Evaluation criterion:

4... Ink-falling does not occur when a 0.3 kilogram weight is used.
3 ... Ink-falling occurs when a 0.25 kilogram weight is used.
2... Ink-falling occurs when a 0.2 kilogram weight is used.
1... Ink-falling occurs when a 0.1 kilogram weight is used.

In addition to the materials and ingredients used in the Examples, other materials and ingredients can be used in the Examples as set forth in the specification to obtain substantially the same results.

As has been described, the thermal transfer recording medium of the present invention does not cause ink-falling when used in low-temperature environments and exerts excellent dot-reproducibility to give printed images with high-definition and excellent durability.

A thermal transfer recording medium which causes no ink-falling and is capable of providing printed images with high definition is disclosed which comprises a substrate having thereon a heat-meltable ink layer, and an intermediate adhesive layer provided between the substrate and the heat-meltable ink layer, the intermediate adhesive layer comprising 20 to 80 % by weight of a resin component consisting of one polyester resin having a glass transition temperature of not higher than 20°C, and 20 to 80 % by weight of at least one component selected from a pigment and carbon black.

## Claims

1. A thermal transfer recording medium comprising a substrate having thereon a heat-meltable ink layer, and an intermediate adhesive layer provided between the substrate and the heat-meltable ink layer, the intermediate adhesive layer comprising 20 to 80 % by weight of a resin component consisting of one polyester resin having a glass transition temperature of not higher than 20 °C, and 20 to 80 % by weight of at least one component selected from a pigment and carbon black.

2. The thermal transfer recording medium of Claim 1, wherein the polyester resin has a glass transition temperature of not higher than 0°C .

3. The thermal transfer recording medium of Claim 1, wherein the heat-meltable ink layer comprises a coloring agent and a vehicle, the vehicle comprising not less than 40 % by weight of caranuba wax.

4. The thermal transfer recording medium of Claim 3, wherein the vehicle comprises not less than 50 % by weight of carnauba wax.

5. The thermal transfer recording medium of Claim 1, wherein the intermediate adhesive layer comprises 40 to 70 % by weight of a polyester resin having a glass transition temperature of not higher than 20°C and 30 to 60 % by weight of at least one of a body pigment and carbon black.

## Patentansprüche

1. Thermisches Übertragungsaufzeichnungsmedium, umfassend ein Substrat mit einer hitzeschmelzbaren Tintenschicht darauf und eine zwischen dem Substrat und der hitzeschmelzbaren Tintenschicht vorgesehene Zwischenhaftschicht, wobei die Zwischenhaftschicht 20 bis 80 Gew.-% einer Harzkomponente, bestehend aus einem Polyesterharz mit einer Glasübergangstemperatur von nicht höher als 20 °C, und 20 bis 80 Gew.-% von mindestens einer Komponente, ausgewählt aus einem Pigment und Ruß, umfaßt.

2. Thermisches Übertragungsaufzeichnungsmedium nach Anspruch 1, wobei das Polyesterharz eine Glasübergangstemperatur von nicht höher als 0 °C besitzt.

3. Thermisches Übertragungsaufzeichnungsmedium nach Anspruch 1, wobei die hitzeschmelzbare Tintenschicht ein Färbemittel und einen Träger umfaßt, wobei der Träger nicht weniger als 40 Gew.-% an Carnaubawachs umfaßt.

4. Thermisches Übertragungsaufzeichnungsmedium nach Anspruch 3, wobei der Träger nicht weniger als 50 Gew.-% an Carnaubawachs umfaßt.

5. Thermisches Übertragungsaufzeichnungsmedium nach Anspruch 1, wobei die Zwischenhaftschicht 40 bis 70 Gew.-% eines Polyesterharzes mit einer Glasübergangstemperatur von nicht höher als 20 °C und 30 bis 60 Gew.-% von mindestens einer Komponente aus einem Substanzpigment und Ruß umfaßt.

## Revendications

1. Support d'enregistrement par transfert thermique comprenant un substrat sur lequel se trouve une couche d'encre thermofusible et une couche adhésive intermédiaire disposée entre le substrat et la couche d'encre thermofusible, la couche adhésive intermédiaire comprenant 20 à 80 % en masse d'un composant résinique consistant en une résine de polyester ayant une température de transition vitreuse qui n'est pas supérieure à 20°C, et 20 à 80 % en masse d'au moins un composant choisi parmi un pigment et le noir de carbone.

2. Support d'enregistrement par transfert thermique selon la revendication 1, dans lequel la résine de polyester a une température de transition vitreuse qui n'est pas supérieure à 0°C.

3. Support d'enregistrement par transfert thermique selon la revendication 1, dans lequel la couche d'encre thermofusible comprend un agent colorant et un véhicule, le véhicule comprenant au moins 40 % en masse de cire de carnauba.

4. Support d'enregistrement par transfert thermique selon la revendication 3, dans lequel le véhicule comprend au moins 50 % en masse de cire de carnauba.

5. Support d'enregistrement par transfert thermique selon la revendication 1, dans lequel la couche adhésive intermédiaire comprend 40 à 70 % en masse d'une résine de polyester ayant une température de transition vitreuse qui n'est pas supérieure à 20°C et 30 à 60 % en masse d'au moins un composant parmi un pigment minéral et le noir de carbone.
